

July 5, 1966

HAJIME NAKAMURA

3,259,488

NITRIDE-BEARING LOW CARBON DUCTILE STEELS

Filed Feb. 10, 1961

8 Sheets-Sheet 1

V-notch charpy transition temperature curve  
and  $T_{715}$  for commercial killed steel.

chemical composition %

| C    | Si   | Mn   | P     | S     |
|------|------|------|-------|-------|
| 0.13 | 0.18 | 0.79 | 0.035 | 0.031 |



FIG. 1      Temperature °C

Shear fracture transition  
temperature curves and  $T_{rs}$   
for commercial killed steel.



FIG. 2      Temperature °C

July 5, 1966

HAJIME NAKAMURA

3,259,488

NITRIDE-BEARING LOW CARBON DUCTILE STEELS

Filed Feb. 10, 1961

8 Sheets-Sheet 2



RELATION BETWEEN TRANSITION TEMPERATURES (CT<sub>15</sub> & TS) AND TOTAL AMOUNT OF ALUMINUM NITRIDE AND ZIRCONIUM NITRIDE CONTAINED IN A NITRIDE-BEARING STEEL

FIG.3



RELATION BETWEEN V-NOTCH CHARPY IMPACT VALUE AND TOTAL AMOUNT OF ALUMINUM NITRIDE AND ZIRCONIUM NITRIDE CONTAINED IN A NITRIDE-BEARING STEEL.

FIG.4

July 5, 1966

HAJIME NAKAMURA

3,259,488

NITRIDE-BEARING LOW CARBON DUCTILE STEELS

Filed Feb. 10, 1961

8 Sheets-Sheet 3

*Solubility curve of AlN in ductile steel B.*



FIG. 5

July 5, 1966

HAJIME NAKAMURA

3,259,488

NITRIDE-BEARING LOW CARBON DUCTILE STEELS

Filed Feb. 10, 1961

8 Sheets-Sheet 4

V-notch charpy transition temperature curve and  
 $T_{75}$  for ductile steel A.  
chemical compositions %

| C    | Si   | Mn   | P     | S     |
|------|------|------|-------|-------|
| 0.10 | 0.32 | 0.59 | 0.016 | 0.023 |

| Al    | N     |
|-------|-------|
| 0.096 | 0.023 |



FIG 6A

Shear fracture transition temperature curve and  
 $T_{rs}$  for ductile steel A.



FIG 7A

July 5, 1966

HAJIME NAKAMURA

3,259,488

NITRIDE-BEARING LOW CARBON DUCTILE STEELS

Filed Feb. 10, 1961

8 Sheets-Sheet 5

V-notch charpy transition temperature curve and  
Tr<sub>15</sub> for ductile steel B.  
chemical composition %

| C    | Si   | Mn   | P     | S     |
|------|------|------|-------|-------|
| 0.08 | 0.23 | 0.57 | 0.016 | 0.021 |

| Al    | N     | Zr   |
|-------|-------|------|
| 0.085 | 0.032 | 0.06 |



FIG 6B

Shear fracture transition temperature curve and  
Tr<sub>s</sub> for ductile steel B.



FIG 7B

July 5, 1966

HAJIME NAKAMURA

3,259,488

NITRIDE-BEARING LOW CARBON DUCTILE STEELS

Filed Feb. 10, 1961

8 Sheets-Sheet 6

V-notch charpy transition temperature curve and  
 $T_{15}$  for ductile steel C.

| C    | Si   | Mn   | P     | S     | Al    |
|------|------|------|-------|-------|-------|
| 0.09 | 0.34 | 0.60 | 0.013 | 0.025 | 0.000 |

| Be    | N      |
|-------|--------|
| 0.019 | 0.0009 |



FIG 6C Shear fracture transition temperature curve and  
 $T_{15}$  for ductile steel C.



FIG 7C

July 5, 1966

HAJIME NAKAMURA

3,259,488

NITRIDE-BEARING LOW CARBON DUCTILE STEELS

Filed Feb. 10, 1961

8 Sheets-Sheet 7

V-notch charpy transition temperature curve and  
 $T_{15}$  for ductile steel D.

chemical composition %

| C    | Si   | Mn   | P     | S     | Al    |
|------|------|------|-------|-------|-------|
| 0.07 | 0.31 | 0.65 | 0.015 | 0.022 | 0.006 |

| Be    | N     |
|-------|-------|
| 0.120 | 0.017 |

FIG 6D

Shear fracture transition temperature curve and  
 $T_{rs}$  for ductile steel D.

FIG 7D



FIG 6D

Shear fracture transition temperature curve and  
 $T_{rs}$  for ductile steel D.

FIG 7D



July 5, 1966

HAJIME NAKAMURA

3,259,488

NITRIDE-BEARING LOW CARBON DUCTILE STEELS

Filed Feb. 10, 1961

8 Sheets-Sheet 8

Changes in mechanical properties of ductile steel quenched from 1200°C and reheated at various temperatures.

chemical composition %

| C    | Si   | Mn   | P     | S     | Cu   | N <sub>2</sub> | Al    | AlN   | Zr   |
|------|------|------|-------|-------|------|----------------|-------|-------|------|
| 0.08 | 0.23 | 0.57 | 0.016 | 0.021 | 0.19 | 0.032          | 0.085 | 0.089 | 0.06 |



FIG. 8

1

3,259,488

### NITRIDE-BEARING LOW CARBON DUCTILE STEELS

Hajime Nakamura, Meguro-ku, Tokyo, Japan, assignor to  
Ishikawajima-Harima Jukogyo Kabushiki Kaisha, Tokyo, Japan, a corporation of Japan  
Filed Feb. 10, 1961, Ser. No. 88,411  
Claims priority, application Japan, Mar. 31, 1960,  
35/11,188, 35/11,189, 35/11,190  
5 Claims. (Cl. 75—124)

This invention relates to nitride-bearing low carbon ductile steels.

More particularly this invention relates to new nitride-bearing low carbon ductile steels containing from 0.015% to 0.090% by weight of a stable nitride selected from the group consisting of beryllium nitride, columbium nitride, a combination of aluminum nitride and beryllium nitride, a combination of aluminum nitride and columbium nitride, a combination of beryllium nitride and columbium nitride and a combination of said three aforesaid nitrides having a certain degree of solubility in the solid state steel at an elevated temperature and/or from 0.01% to 0.10% by weight of another kind of nitride selected from the group consisting of titanium nitride, zirconium nitride and a mixture of both nitrides having practically no solubility in the steel either in the solid and molten states and further less than 0.35% by weight of carbon and if desired, less than 1% by weight of an alloying element selected from the group consisting of nickel, chromium, molybdenum, vanadium, manganese, and silicon.

I discovered that a steel containing nitride or nitrides, a part of which is dissolved in the matrix thereof and another part which exists as free nitride therein, is capable of precipitating out dispersedly its nitride at its grain boundaries and within its grains through the plastic working performed at an elevated temperature, and that such steel with the structure as described above possesses mechanical properties far superior to a steel with the same composition. Particularly, its low temperature toughness is remarkably improved and the transition temperature markedly shifted towards lower temperature.

In the following, I will describe how a low carbon ductile steel with remarkably excellent properties may be produced by the present invention. References will be made to the drawing wherein:

FIG. 1 shows the impact values and Tr15 of a commercial killed steel at various temperatures with respect to three states of as-rolled, as oil-cooled from 950° C. and as air-cooled from 950° C.

FIG. 2 shows the shear fracture ratio and TrS of the same steel.

FIG. 3 represents the relations between the transition temperatures (Tr15 and TrS of a low carbon steel and its sum contents of aluminum nitride and zirconium nitride,

FIG. 4 shows the relation between the impact values of the same steel and its total contents of nitrides,

FIG. 5 shows the solubility curve of aluminum nitride in ductile steel B,

FIGS. 6(A), (B), (C), (D) present impact values and Tr15 of ductile steels A, B, C, D, respectively, in two different states of heat treatment of as oil-cooled from 950° C. and as air-cooled from 950° C.,

FIGS. 7 (A), (B), (C) and (D) show shear fracture

2

ratio and TrS of the same steels as FIGS. 6 (A), (B), (C) and (D), and

FIG. 8 shows the changes in mechanical properties of ductile steel as quenched from 1200° C. and reheated to various temperatures.

Here, the terms Tr15 and TrS signify the temperature at which the energy absorbed in a 2 mm. V-notch Charpy testing specimen reaches the value of 15 ft.-lbs. and the temperature at which shear-fractured portion of the same specimen occupies 50% of the cross-section area of the same specimen, respectively.

If a cast low carbon ductile steel, containing about 0.08% carbon, and 0.090% aluminum nitride precipitated at the grain boundaries in the form of large and long crystals, is subjected to a plastic deformation at a temperature above the  $A_3$  transformation point by a working process such as forging, rolling or like, the crystallites of said steel in as-cast state are broken up and the nitrides present at the grain boundaries may also be finely subdivided, while the former crystallites, on the other hand, tend to grow coarser in general against the breaking action as the temperature is raised to a higher point.

However, the growth of crystallites through the recrystallization process, as described above, is extremely hindered by the fine hard nitride particles that are present within the structure of said finely dispersed steel, thus bringing about a fine crystalline structure to the said steel. It follows that, as the cross-sectional area of the steel is steadily reduced, in other words, as the rolling or forging ratio is increased, by repeated plastic deformation at such an elevated temperature as mentioned earlier, the crystallites of the said steel become finer, and furthermore, as the finishing temperature of rolling or forging is lowered, particularly if such work is done at a temperature range of 1100° C. to 600° C., which corresponds to the maximum precipitation range of the aforementioned nitride, the growth of recrystallized grains is even more inhibited resulting in an even finer granular structure.

It was confirmed by Electronmicroscope technique and X-ray technique that these kinds of nitride that possess certain degrees of solubility in the solid state steel, when precipitated out sufficiently, become as small as 0.1 micron or less.

Thus the strength at both atmospheric and elevated temperature becomes greater while maintaining high impact values, particularly at low temperatures, and the transition temperature becomes extremely shifted to the lower temperature side.

In steels killed with titanium and zirconium in order to decrease the free nitrogen by forming stable compounds with the latter, the action of free nitrogen as a strength raiser is reduced and slip can take place more readily, as a consequence of which, the elongation and reduction of area are remarkably improved and age hardening phenomenon is eliminated. Test results are next presented which show the actual and real improvements in mechanical properties of steels as treated according to the present invention in comparison with those of a commercial killed steel.

Five kinds of steels were prepared for the purpose, as shown in the Table 1, of which steels A and E contain aluminum nitride only, steel B aluminum nitride and zirconium nitride, steels C and D beryllium nitride.

TABLE 1

| Steel           | Chemical Component, Percent |      |      |       |       |                |       |       |       |       |                                |                                |            |       |       |
|-----------------|-----------------------------|------|------|-------|-------|----------------|-------|-------|-------|-------|--------------------------------|--------------------------------|------------|-------|-------|
|                 | C                           | Si   | Mn   | P     | S     | N <sub>2</sub> | Al    | Be    | Zr    | AlN   | Be <sub>3</sub> N <sub>2</sub> | Al <sub>2</sub> O <sub>3</sub> | Soluble Al | ZrN   | CbN   |
| Ductile Steel A | 0.10                        | 0.32 | 0.59 | 0.016 | 0.023 | 0.023          | 0.096 | ----- | 0.06  | 0.071 | -----                          | 0.019                          | 0.087      | 0.02  | ----- |
| Ductile Steel B | 0.08                        | 0.23 | 0.57 | 0.016 | 0.021 | 0.032          | 0.085 | ----- | 0.06  | 0.084 | -----                          | 0.021                          | 0.074      | 0.02  | ----- |
| Ductile Steel C | 0.09                        | 0.34 | 0.60 | 0.013 | 0.025 | 0.009          | 0.006 | 0.119 | ----- | ----- | 0.016                          | -----                          | -----      | 0.024 | ----- |
| Ductile Steel D | 0.07                        | 0.31 | 0.65 | 0.015 | 0.022 | 0.017          | 0.006 | 0.120 | ----- | ----- | 0.024                          | -----                          | -----      | ----- | ----- |
| Ductile Steel E | 0.09                        | 0.27 | 0.55 | 0.014 | 0.023 | 0.021          | 0.038 | ----- | ----- | 0.052 | -----                          | 0.020                          | 0.027      | ----- | ----- |
| Ductile Steel F | 0.09                        | 0.25 | 0.63 | 0.014 | 0.021 | 0.019          | 0.045 | ----- | 0.030 | ----- | 0.011                          | -----                          | 0.06       | ----- | ----- |
| Killed Steel    | 0.13                        | 0.18 | 0.79 | 0.035 | 0.031 | -----          | 0.028 | ----- | 0.009 | ----- | -----                          | -----                          | -----      | ----- | ----- |

The mechanical properties of these steels which have been treated at 950° C. for the precipitation of nitride and then cooled in air, are shown in the Table 2.

themselves under a stressed condition, thereby preventing the dislocations to pile-up at grain boundaries leading to catastrophic crack formation thereat.

TABLE 2

| Steel           | Tensile Strength, kg./mm. <sup>2</sup> | Yield Point, kg./mm. <sup>2</sup> | Yield Ratio, percent | Elongation, percent | Reduction of Area, percent |
|-----------------|----------------------------------------|-----------------------------------|----------------------|---------------------|----------------------------|
| Ductile Steel A | 45.7-46.8                              | 33.3-34.3                         | 72.0-73.5            | 35.4-37.5           | 67.5-71.9                  |
| Ductile Steel B | 41.9-42.2                              | 31.5-33.5                         | 72.6-79.1            | 39.2-40.7           | 77.4-78.4                  |
| Ductile Steel C | 46.5-46.9                              | 32.3-36.9                         | 68.7-78.9            | 37.8-40.0           | 69.8-73.0                  |
| Ductile Steel D | 46.3-47.3                              | 36.3-39.3                         | 76.5-82.7            | 35.0-40.5           | 69.8-73.0                  |
| Ductile Steel E | 43.1-47.3                              | 32.0-33.8                         | 70.5-74.0            | 37.5-39.0           | 71.0-73.5                  |
| Ductile Steel F | 43.7                                   | 36.2                              | 82.8                 | 38.3                | 78.0                       |
| Killed Steel    | 44.0                                   | 30.0                              | 68.2                 | 28.0                | 57.0                       |

FIGS. 1, 2, 6 and 7 compare the sub-zero impact values, Tr15 and TrS of ductile steels due to the present invention with those of a commercial killed steel, in either air-cooled or oil-cooled condition.

The impact value at 0° C., Tr15 and TrS values of ductile steels, as read off these curves, are tabulated in Table 3.

TABLE 3

| Steel           | Impact Value, <sup>1</sup> kg.-m./sq. cm. |                 | Tr15, ° C. |       | TrS, ° C. |      |
|-----------------|-------------------------------------------|-----------------|------------|-------|-----------|------|
|                 | AC <sup>2</sup>                           | OC <sup>3</sup> | AC         | OC    | AC        | OC   |
|                 |                                           |                 |            |       |           |      |
| Ductile Steel A | 30.0                                      | 32.0            | -100       | -125  | -65       | -93  |
| Ductile Steel B | 36.0                                      | 38.0            | -110       | -125  | -82       | -95  |
| Ductile Steel C | 33.0                                      | 33.0            | -95        | -110  | -85       | -90  |
| Ductile Steel D | 32.0                                      | 38.0            | -100       | -110  | -75       | -93  |
| Ductile Steel E | 32.0                                      | 37.0            | -70        | -75   | -40       | -45  |
| Ductile Steel F | 32.0                                      | 438.0           | -100       | 4-120 | -80       | 4-90 |
| Killed Steel    | 15.0                                      | 16.0            | -57        | -70   | -35       | -40  |

<sup>1</sup> Charpy V-notch, at 0° C.

<sup>2</sup> Air-cooled.

<sup>3</sup> Oil-cooled.

<sup>4</sup> Oil-cooled from 930° C. and tempered to 650° C.

FIGS. 3 and 4 show the relation of the total quantity of nitrides to the impact value, Tr15 and TrS. It may be clearly seen that a larger amount of total nitride always corresponds to a higher impact value and lower Tr15 and TrS. It may also be observed that for a steel containing a total amount of nitride over 0.03% up to 0.10%, the low temperature properties are markedly improved.

The result of rupture tests run at 450° C. on ductile steel A indicated a range of duration time of between 88 hours to 125 hours under a stress of 20 kg./mm.<sup>2</sup> with an elongation of between 70% to 80% at rupture, whereas steels with comparable composition but containing no nitride would fail, as judged by the American Society for Testing Materials specifications, after about only 50 hours with an elongation of about 35% to 40% at rupture. This result may be regarded as demonstrating the excellent properties at a high temperature of ductile steels of the present invention.

This exceptionally good high temperature strength may be attributed to the nitride particles which are present in finely dispersed form, in a size as small as 0.1 micron or less, on slip planes of crystallites that restrict the free movement of dislocations by anchoring the latter around

It may be seen from the above experimental results that nitrides are dispersedly precipitated at the grain boundaries and within the grains, and that steels with such a structure exhibit mechanical properties at both atmospheric and elevated temperatures that are far superior to steels of comparable chemical composition but containing no nitride. The improvement in low temperature properties of such nitride-bearing steels is also particularly remarkable.

The present invention relates also to a method of heat treatment for the aforementioned steels containing at least one kind of metallic nitride as described hereinbefore which comprises heating the said nitride-bearing low carbon steel to a temperature above the A<sub>3</sub> transformation point and within such a temperature range that the precipitation of said nitride takes place maintaining at said temperature for a sufficiently long time, so that a large amount of precipitation of said nitride is obtained. The nitride is either aluminum nitride, beryllium nitride, columbium nitride or any combination thereof. Thereafter the said steel is rapidly cooled in air, water or oil while subsequent to the aforementioned process of cooling, the said steel may once again be heated to a temperature below the transformation point for tempering the steel, in order to provide a method of heat treatment for a nitride-bearing ductile steel which not only improves the mechanical properties of the said steel at both room and high temperatures by refining the grain size thereof, but also increases the toughness thereof, particularly at low temperatures, and makes the transition temperature shift towards the lower temperature side.

The heating temperature and holding time may be varied depending on the composition of the steel to be treated, but it is generally preferable to maintain the steel at a temperature above the A<sub>3</sub> transformation point, namely between 800°-1100° C., for a period of time more than 30 minutes.

The tempering is preferably conducted at a temperature between 150°-700° C.

The present heat-treatment method is more fully understood by reference to the drawing.

For example, for a pure iron, low carbon steel or low carbon low alloy steel containing 0.020-0.045% nitrogen, 0.040-0.5% aluminum, 0.05-0.3% zirconium or 0.030-0.1% titanium or both, there may be employed a process comprising heating the said metal to a temperature be-

tween 800° C. to 1100° C. for 30 minutes and, after precipitating the metallic nitride out to the maximum extent, quenching it from a temperature above the  $A_3$  transformation point in air, in oil or in water and subsequently, if desired, tempering at a temperature within a range of 150°-700° C.

For a steel containing 0.005-0.045% nitrogen, 0.01-0.20% beryllium and 0.05-0.20% zirconium or 0.03-0.20% titanium, the process may involve heating at a temperature between 800° C.-1100° C. for less than one (1) hour and then quenching from a temperature above the  $A_3$  transformation point in air, in oil or in water, and further, if preferred, tempering at a temperature between 150°-700° C.

In order to show that the mechanical properties are improved by the process of heat treatment due to the present invention, which involves rapidly cooling or quenching a nitride-bearing ductile steel in a temperature range of most enhanced precipitation for nitrides

the  $A_3$  transformation point, it follows then that a fine grained steel with excellent mechanical properties can be obtained more advantageously by employing both of these processes mentioned above simultaneously rather than by any one of these processes as used singly. That is to say, the present invention relates to a heat treatment method for nitride-bearing steels in which a simultaneous employment of both of these processes described above is featured.

Hereinafter, practical examples of the said method as applied to four (4) kinds of representative ductile steels will be described in detail to show how a nitride-bearing low carbon steel is made to change, improving its structure (ferrite crystal size), room temperature mechanical properties (tensile strength, yield point, elongation, reduction of area, hardness, impact value or like), sub-zero impact values, Tr15, and TrS. Table 4 which contains a part of Table 1 shows the chemical compositions of said steels.

TABLE 4

|                      | C    | Si   | Mn   | P     | S     | Al    | Be    | Zr    | N <sub>2</sub> | AlN   | Be <sub>3</sub> N <sub>2</sub> | ZrN   |
|----------------------|------|------|------|-------|-------|-------|-------|-------|----------------|-------|--------------------------------|-------|
| Ductile Steel A----- | 0.10 | 0.32 | 0.59 | 0.016 | 0.023 | 0.096 | ----- | ----- | 0.023          | 0.071 | -----                          | 0.02  |
| Ductile Steel B----- | 0.08 | 0.23 | 0.57 | 0.016 | 0.021 | 0.085 | 0.06  | 0.06  | 0.032          | 0.087 | -----                          | ----- |
| Ductile Steel C----- | 0.09 | 0.34 | 0.60 | 0.013 | 0.025 | 0.006 | 0.119 | ----- | 0.009          | ----- | 0.016                          | ----- |
| Ductile Steel D----- | 0.07 | 0.31 | 0.65 | 0.015 | 0.022 | 0.006 | 0.120 | ----- | 0.017          | ----- | 0.024                          | ----- |

which lies above the  $A_3$  transformation point, the following is presented, first there is shown the test results of the solubility of nitride in solid state steel, then examples of heat treatment for representative nitride-bearing ductile steels are shown. Namely, nitride-bearing ductile steel containing 0.032% nitrogen was heated for two (2) hours at 1200° C. in order to dissolve the nitride into matrix, then the said nitride was reprecipitated out by heating the said steel at various temperatures between 200° and 1100° C. for one (1) hour at respective temperatures, and then the nitride was chemically separated from the matrix and the amount of nitride was measured. The value thus obtained is to be interpreted as representing a sum of coarser nitride which had already been precipitated out at solid state, namely, that which is insoluble at 1200° C., and finer ones which were newly precipitated in the grains. Therefore, the greater the value, the more the amount of nitrides that have been newly precipitated in the grain is indicated. FIG. 5 illustrates the results of experiments conducted on a steel containing AlN. It may be seen that the precipitation of nitride reaches a maximum at about 700° C. and remains fairly constant up to 1100° C., after which it declines rather rapidly on account of redissolution of the precipitated nitride into the matrix.

It has been established for all the said steels that the ferrite grain size becomes smaller as the cooling rate is increased in order of air-cooling, oil-cooling and water-cooling.

Table 5 presents the grain size of these steels as expressed in terms of the ASTM grain number. It may be seen that extremely fine grain size was attained which hitherto was not possible with a mild steel.

TABLE 5

| 40                   | Steel | ASTM Ferrite Grain Number |      |      |
|----------------------|-------|---------------------------|------|------|
|                      |       | AC                        | OC   | WC   |
| Ductile Steel A----- | ----- | 9                         | 10   | 10.5 |
| Ductile Steel B----- | ----- | 10                        | 10.5 | 11   |
| Ductile Steel C----- | ----- | 10                        | 11   | 11.5 |
| Ductile Steel D----- | ----- | 9                         | 11   | 11   |

It is to be noted that, in each of steels, the ferrite grain number becomes larger in an order of air-cooling, oil-cooling and water-cooling.

Table 6 which is a part of Table 2 shows the tensile strength, yield point, elongation, reduction of area, and Charpy V-notch impact value at -40° C. of the air-cooled steels.

TABLE 6

| Steel                | Tensile Strength, kg./mm. <sup>2</sup> | Yield Point, kg./mm. <sup>2</sup> | Elongation | Reduction of Area, percent | Impact Value*, kg.-m./cm. <sup>2</sup> |
|----------------------|----------------------------------------|-----------------------------------|------------|----------------------------|----------------------------------------|
| Ductile Steel A----- | 45.7-46.8                              | 33.3-34.3                         | 35.4-37.5  | 67.5-71.9                  | 30.0                                   |
| Ductile Steel B----- | 41.9-42.2                              | 31.5-33.5                         | 39.2-40.7  | 77.4-78.4                  | 36.0                                   |
| Ductile Steel C----- | 46.5-46.9                              | 32.3-36.9                         | 37.8-40.0  | 69.8-73.0                  | 33.0                                   |
| Ductile Steel D----- | 46.3-47.5                              | 36.9-39.3                         | 35.0-40.5  | 69.8-73.0                  | 30.7                                   |

\*Charpy 2 mm. V-notch, at -40° C., in kg.-m./cm.<sup>2</sup>.

Similar relationships were also observed on steels containing beryllium nitride.

Therefore, when the improvement of the mechanical properties of steels is to be realized by virtue of the precipitation of nitride only, this may be achieved by heating the said steel to a temperature below the transformation point for a sufficiently long period of time, but as the granular structure of a steel can be refined by rapidly cooling it from a temperature immediately above

70 of these steels, one with less than 0.01% carbon, namely a very mild steel, exhibits almost no change by air-cooling or oil-cooling thereby needing no tempering, yet, such a steel, too, can be made ductile by the method of the present invention so as to be a structural steel in sufficiently low temperatures.

FIGS. 6 and 7 represent the comparison of sub-zero impact values, Tr15 and TrS between representative ductile steels described above as obtained according to air-

cooled and oil-cooled operations, respectively, to show that, in any one of the cases, oil-cooled steels exhibit better properties than those that are air-cooled. Though no particular emphasis is needed, it may be stated here that these steels in merely an air-cooled state are superior to those in as-annealed, as-rolled or as-forged conditions.

The above results are summarized in the following Table 7 which is a part of Table 3.

TABLE 7

| Steel                | Impact Value,*<br>kg.-m./cm. <sup>2</sup> |       | Tr15, ° C. |       | TrS, ° C. |      |
|----------------------|-------------------------------------------|-------|------------|-------|-----------|------|
|                      | AC                                        | OC    | AC         | OC    | AC        | OC   |
| Ductile Steel A----- | 30.0                                      | 32.0  | -100       | -125  | -65       | -90  |
| Ductile Steel B----- | 36.0                                      | 38.0  | -110       | -125  | -80       | -95  |
| Ductile Steel C----- | 33.0                                      | 33.0  | -95        | -110  | -80       | -90  |
| Ductile Steel D----- | 31.0                                      | 37.0  | -100       | -110  | -70       | -90  |
| Ductile Steel F----- | 32.0                                      | †38.0 | -100       | †-120 | -80       | †-90 |

\*Maximum value, Charpy 2 mm. V-notch, at ° C.  
†Oil-cooled and tempered.

Steels containing more than 0.10% carbon tend to harden somewhat by quenching, and as a result, the tensile strength, yield point, and hardness are slightly raised, while the elongation, reduction of area and impact values suffer a reduction. This means the process of tempering become necessary for such steels following the water-cooling. FIG. 8 shows the change in tensile strength, yield point, hardness, elongation, reduction of area and impact value of ductile steel A as the said steel is tempered at various temperatures above 200° C. following quenching from 1100° C.

It may be seen that the tensile strength and yield point are reduced rather sharply at 400° C.; the elongation is almost recovered at about 300° C. and is improved still further as the tempering temperature is raised; while, the reduction of area and impact value are completely recovered at about 300° C. and no noticeable further gain is observed at a higher temperature.

It may be stated on the strength of these experimental results described above that the mechanical properties of ductile steel can be improved by rapidly cooling the said steel from a temperature within the range of maximum nitride precipitation and above the A<sub>3</sub> transformation point, and that such steel becomes an excellent structural steel for low temperature service with its Tr15 and TrS, both of which are known to represent well the low temperature ductility, and are markedly shifted towards the lower temperature side.

more stable nitrides, in order to convert the excessive nitrogen into nitride or nitrides of the aforementioned metal or metals, and if desired, heat treating the steel thus produced in order to precipitate out a part of the nitride, and then subjecting the steel to a plastic deformation at an elevated temperature such as by rolling or forging.

The steels utilized in this process are pure iron, low carbon steels with approximately 0.35% carbon or less, or low carbon low alloy steels containing alloying elements other than carbon by less than 1.0% each.

I have found that when from 0.015 to 0.09% of nitride or nitrides of metal or metals such as aluminum, beryllium, columbium or the like are present in a steel, the said steel possesses superior mechanical properties at atmospheric and elevated temperatures, particularly as regards its impact strength at low temperatures while the transition temperature is remarkably shifted towards the lower temperature side, as compared to a steel with the same components except the nitride.

The nitride-bearing steel may be successfully produced using any one of an over-blowing converter, open-hearth furnace, electric arc furnace, or high-frequency electric furnace and the production method can be categorized into two categories, as now will be described more fully

The first category concerns the blowing into molten steel of nitrogen gas or a mixed gas composed of nitrogen and a gas or gases that is inert to the steel (for example, a mixed gas of nitrogen and argon, helium or the like), subsequently adding to the steel one, or more than one kind of a metal that reacts with the nitrogen to form a hard nitride having a certain degree of solubility in the solid state steel, such metals may be aluminum, beryllium, or columbium. These metals react with the aforementioned nitrogen, making the said steel a nitride-bearing ductile steel. One practical example of producing ductile steel in an electric arc furnace by means of a process mentioned above is now described in detail.

#### Example 1

Firstly, scrap steel was melted by an electric arc furnace and refined under an oxidizing condition, then 0.35% of ferro-silicon and 0.70% of ferromanganese were added for deoxidation, then nitrogen gas was blown into the molten steel through a conduit pipe for about 6 minutes at a pressure of 5 kg., following which 0.20% of aluminum in one case and 0.10% beryllium in the other was added prior to the casting of the steel into ingots. The Table 8 shows the chemical composition of two (2) representative steels produced by the aforementioned process.

TABLE 8

| Steel  | C    | Si   | Mn   | P     | S     | N <sub>2</sub> | Al    | AlN   | Al <sub>2</sub> O <sub>3</sub> | Be    | Be <sub>3</sub> N <sub>2</sub> |
|--------|------|------|------|-------|-------|----------------|-------|-------|--------------------------------|-------|--------------------------------|
| G----- | 0.07 | 0.25 | 0.61 | 0.015 | 0.022 | 0.035          | 0.15  | 0.088 | 0.020                          | 0.120 | 0.024                          |
| H----- | 0.07 | 0.31 | 0.65 | 0.015 | 0.022 | 0.015          | 0.006 |       |                                |       |                                |

As may be seen, a part of the aluminum added is combined with oxygen that was present in the molten steel and becomes aluminum oxide, while the rest is formed as aluminum nitride. Also, the beryllium nitride, Be<sub>3</sub>N<sub>2</sub>, was clearly shown by the chemical analysis.

Nextly, ingots thus produced were brought to a temperature between 1150° C. and 1250° C., which corresponds to a state where the nitride exists partially as dissolved and partially as solid phase, and the ingots were forged thereat with a finishing temperature 850° C. The steel was left to cool to atmospheric temperature, subsequent to which the said steel was heated again at 950° C. for one (1) hour, and then again cooled in air. Table 9 compares the mechanical properties of steels produced by the above method and of a commercially available high killed mild steel with a comparable chemical composition.

TABLE 9

| Steel                   | Tensile Strength, kg./sq. mm. | Yield Point, kg./sq. mm. | Elongation, percent | Reduction of Area, percent | Impact Value, <sup>2</sup> kg.-m./sq. cm. | Tr15, °C. | TrS, °C. |
|-------------------------|-------------------------------|--------------------------|---------------------|----------------------------|-------------------------------------------|-----------|----------|
| G-----                  | 42.0                          | 32.0                     | 40.0                | 79.0                       | 35.5                                      | -105      | -85      |
| H-----                  | 46.7                          | 38.0                     | 39.0                | 71.0                       | 31.0                                      | -100      | -70      |
| Mild Steel <sup>1</sup> | 44                            | 30                       | 28                  | 57                         | 8.0                                       | -47       | -30      |

<sup>1</sup> 0.13% C, killed.<sup>2</sup> At 0°C.

Therefore, it can be stated that the present method is fully capable of producing a nitrogen-bearing ductile steel.

Furthermore, this process of nitrogen blowing has an additional effect of obtaining cleaner steel by virtue of the stirring action the nitrogen gas induces within the molten metal, thus stimulating various deoxidization products that are present therein to coagulate.

If a nitride-bearing steel is to be produced by the aforementioned process only, the ingot is not stabilized, or killed, and becomes a so-called rimmed ingot containing blow holes within, since an amount of nitrogen gas that is left uncombined tries to escape therefrom as the metal solidifies. However, even this kind of ingot provides no disadvantage when offered for sale, as far as the quality of the steel is concerned, since the aforementioned blow holes can readily be eliminated during forging or rolling.

However, killed steels are often more desirable when higher quality ingots are desired. In order to achieve this purpose, it calls for use in a general practice of a quantity of aluminum as much as about 1%, when used singly to bring forth a change in the properties of the steel.

I have succeeded in stabilizing, or killing, the nitride-bearing ductile steel by fixing the excessive nitrogen gas that is escaping therefrom at its solidification by means of a metal or metals that can form even more stable nitride or nitrides than those of aluminum or beryllium and that do not dissociate at a solidification temperature of the steel. Of metals with the aforementioned property, titanium and zirconium were found to be most suitable, and an addition of about 0.03% to 0.3% thereof was seen to be sufficient to achieve the purpose. The titanium nitride and zirconium nitride resulting herein are all insoluble in the molten steel, one part of which is eliminated therefrom, while the rest which is floating therein, become finely and dispersedly suspended therein as the steel solidifies; the particles of said metallic nitride in a form as described above have no adverse effects on the steel, and even a favorable influence could be expected for the steel.

In Table 10 are represented the chemical composition and mechanical properties of a steel produced through the process described above.

TABLE 10

| Steel   | C                             | Si                          | Mn                  | P                          | S                                         | N <sub>2</sub> | Al       | Zr   | AlN   | Al <sub>2</sub> O <sub>3</sub> | ZrN  |
|---------|-------------------------------|-----------------------------|---------------------|----------------------------|-------------------------------------------|----------------|----------|------|-------|--------------------------------|------|
| B*----- | 0.08                          | 0.23                        | 0.57                | 0.016                      | 0.021                                     | 0.032          | 0.085    | 0.06 | 0.084 | 0.021                          | 0.02 |
| Steel   | Tensile Strength, kg./sq. mm. | Yield Strength, kg./sq. mm. | Elongation, percent | Reduction of Area, percent | Impact Value, <sup>†</sup> kg.-m./sq. cm. | Tr15, °C.      | TrS, °C. |      |       |                                |      |
| B*----- | 41.0-42.2                     | 31.5-33.5                   | 39.2-40.7           | 77.4-78.4                  | 36.0                                      | -100           | -80      |      |       |                                |      |

<sup>†</sup>Ductile steel.<sup>†</sup>At 0°C.

It may be seen that the fixation of free nitrogen by means of adding such metallic element like zirconium or titanium is evidently effective for producing killed ductile steel.

The second method comprises blowing the calcium cyanamide into the molten steel together with an inert gas (for example, argon) or nitrogen gas or a mixed gas consisting of nitrogen and an inert gas, so that nitrogen is introduced therewith as a result of direct reaction of gaseous nitrogen, and subsequent to the above, an amount of metallic element or elements that yield the desired nitride as before is introduced, thus rendering the steel nitride-bearing and ductile.

I therefore particularly point out and distinctly claim as my invention:

1. A nitride-bearing ductile steel consisting of less than 0.35% carbon, less than 0.035% of each of sulphur and phosphorus, less than 1% of manganese, less than 0.5% of silicon, from 0.015 to 0.090% of at least one of the substances selected from the group consisting of beryllium nitride, columbium nitride, a combination of aluminum nitride and beryllium nitride, a combination of aluminum nitride and columbium nitride, a combination of beryllium nitride and columbium nitride, and a combination of aluminum nitride, beryllium nitride and columbium nitride; from 0.01 to 0.10% of at least one of the nitrides selected from the group consisting of titanium nitride and zirconium nitride, the remainder being substantially all iron with incidental impurities, a portion of the nitrides being combined in the matrix of the steel, the remainder of the nitrides existing as free nitride in the form of fine particles dispersedly precipitated in the grains and on the grain boundaries of the steel to thereby provide improved mechanical properties for the steel.

2. A nitride-bearing ductile steel consisting of less than 0.35% carbon, less than 0.035% of each of sulphur and phosphorus, less than 1% of manganese, less than 0.5% of silicon, from 0.015 to 0.090% of the substances selected from the group consisting of; beryllium nitride, columbium nitride, a combination of aluminum nitride and beryllium nitride, a combination of aluminum nitride and columbium nitride, a combination of beryllium nitride and columbium nitride, a combination of aluminum nitride, beryllium nitride and columbium nitride, from 0.01% to 0.10% of at least one of the nitrides selected from the group consisting of titanium nitride and zirconium nitride less than 1.0% of at least one of the elements selected from the group consisting of nickel,

chromium, vanadium, and molybdenum; less than 0.5% boron, the remainder being substantially all iron with incidental impurities, a portion of the nitrides being combined in the matrix of the steel, the remainder of the

nitrides existing as free nitride in the form of fine particles dispersedly precipitated in the grains and on the grain boundaries of the steel to thereby provided improved mechanical properties for the steel.

3. A nitride-bearing ductile steel consisting of less than 0.35% carbon, less than 0.5% silicon, less than 1.0% of at least one of the elements selected from the group consisting of manganese, nickel, chromium, vanadium, and molybdenum, less than 0.5% boron, from 0.015 to 0.090% aluminum nitride and from 0.01 to 0.10% of at least one of the nitrides selected from the group consisting of titanium nitride and zirconium nitride, the remainder being substantially all iron with incidental impurities, a portion of the nitrides being combined in the matrix of the steel, the remainder of the nitrides existing as free nitride in the form of fine particles dispersedly precipitated in the grains and on the grain boundaries of the steel to thereby provide improved mechanical properties for the steel.

4. A nitride-bearing ductile steel consisting of less than 0.35% carbon, less than 0.35% of each of sulphur and phosphorus, less than 1% of manganese, less than 0.5% of silicon, from 0.015 to 0.090% of at least one of the substances selected from the group consisting of beryllium nitride, columbium nitride, a combination of aluminum nitride and beryllium nitride, a combination of aluminum nitride and columbium nitride, a combination of beryllium nitride and columbium nitride, and a combination of aluminum nitride, beryllium nitride and columbium nitride, the content of beryllium nitride being from 0.015 to 0.065%; from 0.01 to 0.10% of at least one of the nitrides selected from the group consisting of titanium nitride and zirconium nitride, the remainder being substantially all iron with incidental impurities.

5. A nitride-bearing ductile steel consisting of less than 0.35% carbon, less than 0.035% of each of sulphur and phosphorus, less than 1% of manganese, less than 0.5% of silicon, from 0.015 to 0.090% of at least one of the substances selected from the group consisting of beryllium nitride, columbium nitride, a combination of aluminum nitride and beryllium nitride, a combination of aluminum nitride and columbium nitride, a combination of beryllium nitride and columbium nitride, and a combination of aluminum nitride, beryllium nitride and columbium nitride, the content of columbium nitride being from 0.035 to 0.090%; from 0.01 to 0.10% of at least one of the nitrides selected from the group consisting of titanium nitride and zirconium nitride, the remainder being substantially all iron with incidental impurities.

#### References Cited by the Examiner

##### UNITED STATES PATENTS

|           |         |                     |         |    |
|-----------|---------|---------------------|---------|----|
| 2,174,740 | 10/1939 | Graham et al. ----- | 75—123  | XR |
| 2,482,948 | 9/1949  | Sykes et al. -----  | 75—129  |    |
| 2,501,138 | 3/1950  | Parker -----        | 75—129  |    |
| 2,562,543 | 7/1951  | Gippert -----       | 75—123  |    |
| 2,563,672 | 8/1951  | Boyce -----         | 148—134 |    |
| 2,602,736 | 7/1952  | Sheridan -----      | 75—123  |    |
| 2,603,562 | 7/1952  | Rapatz -----        | 75—123  |    |
| 2,938,820 | 5/1960  | Turner -----        | 148—134 |    |

##### FOREIGN PATENTS

|    |         |        |        |
|----|---------|--------|--------|
| 30 | 530,500 | 8/1955 | Italy. |
|----|---------|--------|--------|

DAVID L. RECK, Primary Examiner.

RAY K. WINDHAM, MARCUS U. LYONS, Examiners.

R. O. DEAN, Assistant Examiner.